

# UNITED STATES PATENT OFFICE.

ALEXANDER JOHNSTON AGNEW AND FRANK FORSTER RENWICK, OF ILFORD, ENGLAND, ASSIGNORS TO ILFORD LIMITED, OF ILFORD, ENGLAND.

## HIGH-TEMPERATURE DEVELOPMENT OF PHOTOGRAPHIC MATERIALS.

1,424,062.

Specification of Letters Patent.

Patented July 25, 1922.

No Drawing.

Application filed February 28, 1919. Serial No. 279,882.

To all whom it may concern:

Be it known that we, ALEXANDER JOHNSTON AGNEW and FRANK FORSTER RENWICK, subjects of the King of England, and both

5 residing at Ilford, in the county of Essex, England, have invented certain new and useful Improvements in High-Temperature Development of Photographic Materials, of which the following is a specification.

10 This invention is for improvements in or relating to high-temperature development or other treatment by aqueous solutions of photographic materials, and has for its object to provide a process whereby these 15 materials may be safely manipulated in tropical countries, or in abnormally hot weather elsewhere.

Special developers have heretofore been proposed for developing in these circumstances, but such developers have usually a strong tendency to fog, the development is so rapid that it cannot be conveniently controlled, and they are of little use at a temperature of 90° F. or over.

20 According to the present invention, a hardening bath or mixture is provided for treating gelatine-surfaced photographic materials prior to subjecting them to the action of a developer or other aqueous solution, which bath contains formaldehyde solution, paraform, or a compound from which formaldehyde is readily obtained, together with a salt (for example, sodium citrate or sodium sulphate or di-sodium 25 ortho-phosphate) of the known class which tends to raise the melting point of a gelatine jelly and to retard or restrict the swelling of dry gelatine in water.

The invention further consists in the 30 process for developing or otherwise treating by aqueous solutions gelatine-surfaced photographic materials at high temperatures consisting in first subjecting the material to a hardening bath such as above described, 35 and then subjecting it to a developer or other aqueous solution. It is found that if a photographic plate, for example, be first hardened in the aforesaid manner, it can afterwards be developed or say toned with 40 ease by any of the known developers or toning baths at a high temperature.

The class of salts referred to includes acetates, tartrates, citrates, oxalates, sulphates, phosphates, chromates, bicarbonates, and borates.

55 A formula for this preliminary bath may be as follows:—

|                             |             |
|-----------------------------|-------------|
| 40% formaldehyde solution   | 10 c. c. m. |
| Sodium sulphate crystals    | 80 grams.   |
| Or di-sodium orthophosphate | 40 grams.   |
| Water up to                 | 400 c. c.   |

60 or if paraform be employed 4.5 grams of this may be used instead of the 10 c. c. of formaldehyde solution.

65 The above formula may be compounded and kept indefinitely, or the paraform and sodium sulphate or other salt in anhydrous form may be made up as powders or into pellets and sold in this condition for dissolving when required in the necessary quantity of water.

70 It will be appreciated that the formula for the purpose of this invention may be variously modified without departing from the 75 spirit of the invention, various salts other than sodium sulphate being available as already described. Almost any base may be employed that will give a soluble salt though all are not equally good but besides sodium 80 salts ammonium and magnesium have been found to give good results.

85 It has been found that by using this preliminary bath, photographic plates and other materials can be manipulated that is developed, toned, fixed, washed or otherwise treated with aqueous solutions at a temperature as high as 110° F. without any cooling means being necessary. The salt retards the swelling and prevents melting of the 90 gelatine while the formaldehyde solution is penetrating and combining with it to form an insoluble film, so that even though the bath may be as high a temperature as 110° F. the gelatine has no opportunity to melt 95 before it is hardened by the formaldehyde solution.

100 The advantage of using the above ingredients as a preliminary bath to a developing bath is great as it disposes of the need of using a special developer. Further, the fact that no development is taking place during

this hardening, enables the developing to be carried out afterwards without undue haste, whereas when the hardening material has been incorporated in the developer, the 5 hardening action has scarcely begun before development is finished and this is so rapid that, as already stated, it cannot be controlled; moreover, the hardening effect being imperfect, subsequent treatment, such as fixing and washing of the plate is exceedingly difficult and at such temperatures as 100° to 110° F. it is impossible even to complete development itself before the gelatine melts. When, however, the hardening is effected in 10 a preliminary bath as described, the developing and fixing and washing can all be subsequently carried out in practically the same manner and with almost as much ease as would be the case if operating in ordinary 15 temperatures.

The advantages referred to above as the result of applying this invention to developing also accrue in part to other manipulations such as toning.

20 25 It will be understood that the invention is applicable to all gelatine-surfaced photographic materials, such for example as plates, papers, and films.

In practice it is usual to proceed with development immediately after rinsing off the 30 excess of the preliminary hardening bath.

What we claim as our invention and desire to secure by Letters Patent is:—

35 40 45 1. A composition for treating gelatine-surfaced photographic materials for hardening them only, comprising a substance adapted to yield formaldehyde together with a relatively greater amount of a salt of the known class which tends to raise the melting point of a gelatine jelly and to retard or restrict the swelling of gelatine in water.

2. A composition for treating gelatine-surfaced photographic materials for hardening them only, comprising a substance adapted to yield formaldehyde together with a salt of the known class which tends to raise the melting point of a gelatine jelly and to retard or restrict the swelling of gelatine in 50 water, in concentration in excess of one molecular proportion relatively to the formaldehyde yielding substance to preserve the consistency of the gelatine surface pending reaction therewith of the formaldehyde.

55 60 65 3. A composition for treating gelatine-surfaced photographic materials for hardening them only, comprising a substance adapted to yield formaldehyde together with an alkali salt of the known class which tends to raise the melting point of a gelatine jelly and to retard or restrict the swelling of gelatine in water, in concentration in excess of one molecular proportion relatively to the formaldehyde yielding substance to preserve

the consistency of the gelatine surface pending reaction therewith of the formaldehyde.

4. A composition for treating gelatine-surfaced photographic materials for hardening them only, comprising a substance adapted to yield formaldehyde together with 70 a sodium salt of the known class which tends to raise the melting point of a gelatine jelly and to retard or restrict the swelling of gelatine in water, in concentration in excess of one molecular proportion relatively to the 75 formaldehyde yielding substance to preserve the consistency of the gelatine surface pending reaction therewith of the formaldehyde.

5. A composition for treating gelatine-surfaced photographic materials for hardening them only, comprising a substance adapted to yield formaldehyde together with sodium citrate in such concentration as to 80 preserve the consistency of the gelatine surface 85 pending reaction therewith of the formaldehyde.

6. A composition for treating gelatine-surfaced photographic materials for hardening them only, comprising a solution of free 90 formaldehyde together with a salt of the known class which tends to raise the melting point of a gelatine jelly and to retard or restrict the swelling of gelatine in water in such concentration as to preserve the 95 consistency of the gelatine surface pending reaction therewith of the formaldehyde.

7. A composition for treating gelatine-surfaced photographic materials for hardening them only, comprising a solution of free 100 formaldehyde together with an alkali salt of the known class which tends to raise the melting point of a gelatine jelly and to retard or restrict the swelling of gelatine in water in such concentration as to preserve 105 the consistency of the gelatine surface pending reaction therewith of the formaldehyde.

8. A composition for treating gelatine-surfaced photographic materials for hardening them only, comprising a solution of free 110 formaldehyde together with a sodium salt of the known class which tends to raise the melting point of a gelatine jelly and to retard or restrict the swelling of gelatine in water, in such concentration as to preserve 115 the consistency of the gelatine surface pending reaction therewith of the formaldehyde.

9. A composition for treating gelatine-surfaced photographic materials for hardening them only, comprising a solution of 120 free formaldehyde together with sodium citrate in such concentration as to preserve the consistency of the gelatine surface pending reaction therewith of the formaldehyde.

10. A process for hardening gelatine-surfaced photographic materials comprising subjecting the material to treatment in a bath comprising formaldehyde together with

a salt of the known class which tends to raise the melting point of a gelatine jelly and to retard or restrict the swelling of gelatine in water in such concentration as to preserve the consistency of the gelatine surface pending reaction therewith of the formaldehyde.

5 In testimony whereof we have signed our

names to this specification in the presence of two subscribing witnesses.

ALEXANDER JOHNSTON AGNEW.  
FRANK FORSTER RENWICK.

Witnesses:

A. M. HARWARD,  
HARRY S. LINDGE.